

## UNITED STATES PATENT OFFICE

2,010,176

## WETTING ASSISTANT FOR MERCERIZING COTTON

Karl Brodersen, Dessau in Anhalt, Germany, assignor to General Aniline Works, Inc., New York, N. Y., a corporation of Delaware

No Drawing. Application September 10, 1931,  
Serial No. 562,206. In Germany September 24,  
1930

12 Claims. (Cl. 8—20)

My present invention relates to new wetting agents and more particularly to products to be used as assistants in the mercerization of cotton.

5 I have found that those ethers of polyhydric alcohols which contain at least two free hydroxy groups in the molecule, are valuable wetting agents for mercerizing lyes.

The compounds in question generally correspond to the formula



15 wherein A means an aliphatic radicle containing at least three carbon atoms, R means an aliphatic radicle containing less than six carbon atoms, x stands for 2 or a whole number greater than 2 and y stands for 1 or a whole number greater than 1.

20 The ethers, particularly suitable in this respect, are the propyl ether, butyl ether, isobutyl

to act upon an equimolecular amount of the sodium compound of monohydric alcohols. The ethers need not be prepared in a chemically pure state; the raw products obtainable according to the process set forth already yield the desired result.

5 The ethers employed in the process are nearly colorless oils which are soluble in water and have a faint odor. They readily dissolve in mercerizing lyes, part of them with a feeble opalescence. 10 Their aqueous solutions have no wetting power at all, this being brought out only in strong caustic alkali solutions. Therefore, when added to mercerizing lyes, the effect produced by these agents is that the material to be mercerized is 15 more rapidly soaked with the liquor so that a much more rapid and more uniform shrinking of the yarn or of the tissue is produced.

The effect of the process of this invention may be seen from the following comparative tests:

20 Hanks of cotton yarn are immersed in a mercerizing liquor of 30° Bé. and about 20° C.

| 25                 | Kind of yarn | Addition to the liquor                 | Percentage of the shrinking of the original length after |      |      |      |      |      | 25 |  |
|--------------------|--------------|----------------------------------------|----------------------------------------------------------|------|------|------|------|------|----|--|
|                    |              |                                        | Seconds                                                  |      |      |      |      |      |    |  |
|                    |              |                                        | 20                                                       | 40   | 60   | 80   | 100  | 120  |    |  |
| 30                 |              |                                        |                                                          |      |      |      |      |      | 30 |  |
| Boiled cotton yarn |              |                                        | 10.5                                                     | 12.8 | 12.9 | 13   | 13   | 13   |    |  |
| Crude cotton yarn  |              |                                        | 0.4                                                      | 1.4  | 2.5  | 3.5  | 4.3  | 5    |    |  |
| Crude cotton yarn  |              | Glycerinmono-butylether 1 g. per liter | 4.5                                                      | 10.5 | 13.9 | 15.8 | 16.7 | 17.5 |    |  |
| Crude cotton yarn  |              | Glycerinmono-butylether 2 g. per liter | 13.5                                                     | 16.8 | 16.9 | 17   | 17   | 17   |    |  |
| Crude cotton yarn  |              | Glycerinmono-amylether 2 g. per liter  | 13                                                       | 16.8 | 16.3 | 16.5 | 16.5 | 16.5 | 35 |  |

ether, the different amyl and hexyl ethers of polyhydric alcohols with at least two free OH groups in the alcoholic radicle and more specifically such compounds which contain in summa 6 to 10 carbon atoms. As polyhydric alcohol from which the ethers derive, glycerin is best suited on account of its ready accessibility and its property to be easily etherified in one OH group; there can, however, also be employed corresponding esters of higher polyhydric alcohols such as, for instance, sorbite and those alcohols whose carbon chain is interrupted, for instance, by oxygen bridges, such as diglycerine.

45 As representants of the preferred group I enumerate monopropyl glycerin ether, monobutyl- and isobutyl glycerin ether and the different monoamyl glycerin ethers. These monoethers may be prepared by causing the monochlorhydrines of the corresponding polyhydric alcohols

40 The wetting power of my assistance is clearly shown in the foregoing table from the accelerated action of the strong caustic alkali lye which manifests itself in the shrinkage of the yarn. Thus, the degree of the wetting capacity is indicated in this table by the percentage of shrinking in the units of time.

45 The amount of each assistant I add to the mercerizing lye may vary in certain limits. A good effect is obtainable when adding about 1 gram of a monoether of the kind described per liter of the lye; the quantity of the additional substance may be raised up to 5 grams per liter, 50 however, generally a satisfying effect is reached with 2 to 3 grams per liter.

55 What I claim is:

1. A process for mercerizing cotton which comprises submitting it to the action of a preparation

5

10

15

20

25

30

35

40

45

50

55

consisting of an alkali lye and a compound which corresponds to the general formula



wherein A means an aliphatic radicle containing at least three carbon atoms, R means an aliphatic radicle containing less than six carbon atoms, x stands for 2 or a whole number greater than 2, 10 and y stands for 1 or a whole number greater than 1.

2. A process for mercerizing cotton which comprises submitting it to the action of a preparation 15 consisting of an alkali lye and a compound which corresponds to the general formula



wherein R stands for an aliphatic radicle containing less than six carbon atoms.

3. A process for mercerizing cotton which comprises submitting it to the action of a preparation 25 consisting of an alkali lye and a glycerin-monopropyl ether.

4. A process for mercerizing cotton which comprises submitting it to the action of a preparation 30 consisting of an alkali lye and a glycerin-monobutyl ether.

5. A process for mercerizing cotton which comprises submitting it to the action of a preparation 35 consisting of an alkali lye and a glycerin-monoamyl ether.

6. A process for mercerizing cotton which comprises submitting it to the action of a preparation 40 consisting of an alkali lye and a compound which corresponds to the general formula



wherein R stands for propyl, butyl or amyl.

7. A mercerizing lye consisting of a caustic alkali and a compound of the general formula



wherein A means an aliphatic radicle containing at least three carbon atoms, R means an aliphatic radicle containing less than six carbon atoms, x 10 stands for 2 or a whole number greater than 2, and y stands for 1 or a whole number greater than 1.

8. A mercerizing lye consisting of a caustic alkali and a compound of the general formula 15



5

20

wherein R stands for an aliphatic radicle containing less than six carbon atoms.

9. A mercerizing lye consisting of a caustic alkali and a glycerinmonopropyl ether.

10. A mercerizing lye consisting of a caustic alkali and a glycerinmonobutyl ether.

11. A mercerizing lye consisting of a caustic alkali and a glycerinmonoamyl ether.

12. A mercerizing lye consisting of a caustic alkali and a compound of the general formula



35

40

wherein R stands for propyl, butyl or amyl.

KARL BRODERSEN.